# EUROPEAN PATENT APPLICATION

(11) **EP 4 484 530 A1**
(43) Date of publication of application: **01.01.2025**
(21) Application number: 23182187.7
(22) Date of filing: 28.06.2023
(51) Int. Cl.: C11D 1/22, C11D 17/06, C11D 11/04

(54) **A SOLID LINEAR ALKYL BENZENE SULPHONATE ANIONIC DETERSIVE SURFACTANT PARTICLE**

(71) Applicant: The Procter & Gamble Company, Cincinnati, OH 45202 (US)
(72) Inventor: BESIRIK, Olgun, Newcastle upon Tyne, NE12 9BZ (GB); GRAHAM, Stephanie Kate, Newcastle upon Tyne, NE12 9BZ (GB); TANTAWY, Hossam Hassan, Newcastle upon Tyne, NE12 9BZ (GB)
(74) Representative: P&G Patent Belgium UK

(57) **Abstract**

The present invention relates to a solid linear alkyl benzene sulphonate anionic detersive surfactant particle. The particle contains a polycationic salt of linear alkyl benzene sulphonic acid having both magnesium and sodium cations. The weight ratio of the magnesium salt of linear alkyl benzene sulphonic acid to the sodium salt of linear alkyl benzene sulphonic acid is in the range of from 0.6: 1 to 9:1.

## Description

### FIELD OF THE INVENTION

The present invention relates to a solid linear alkyl benzene sulphonate anionic detersive surfactant particle. The particle contains a polycationic salt of linear alkyl benzene sulphonic acid having both magnesium and sodium cations. The weight ratio of the magnesium salt of linear alkyl benzene sulphonic acid to the sodium salt of linear alkyl benzene sulphonic acid is carefully controlled. The particle has a good storage stability and a good dissolution upon contact with water.

### BACKGROUND OF THE INVENTION

Laundry detergent manufacturers formulate products with surfactants as the core chemistry to provide fabric cleaning during washing. One such surfactant category comprises anionic linear alkylbenzene sulphonates (LAS), which can be delivered in a number of physical forms. For the manufacture of solid powder detergents, these forms typically comprise a spray-dried particle, an agglomerated particle, or a flaked particle. Which of these forms is used typically depends on factors such as but not limited to the surfactant activity of the particle, the cost to manufacture the particle, the rate at which the particle can be produced, the physical properties of the particle, and/or any combination of these and/or other factors.

A large majority of the solid powder detergent industry provides LAS in the form of either spray-dried particles or agglomerated particles. These particles are generally limited by a maximum mass of LAS per mass of particle - i.e., the particle activity - in terms of their ability to be manufactured or the physical properties of the final particle. Higher active LAS particles tend to be more difficult to process due to the adhesive nature of LAS, especially in humid conditions. It is typically observed that increasing the activity of an LAS particle reduces the humidity at which handling issues are seen. As it is the desire of the industry to move into more concentrated formulations to reduce the carbon footprint of its applications, higher active surfactant particles become more and more attractive, which magnifies the challenge around providing consumers with a free-flowing powder detergent formulation.

The highest active LAS particles commercially available currently are so-called LAS flakes, which have an activity typically exceeding 80%w LAS. As such, they are particularly susceptible to moisture. The inventors have found that changing the counter-ion of the LAS species affects the sensitivity of the LAS to moisture, particularly the effect of (the amount of present) moisture on its physical properties such as bulk flow. High-active MgLAS₂ particles were observed to maintain their free-flowing properties up to a higher degree of moisture presence (measured as the particles' relative humidity) compared to their NaLAS counterparts.

The inventors have also found that the dissolution kinetics of MgLAS₂ particles are inferior to their NaLAS counterparts. However, the inventors have found that the negative cohesive properties of NaLAS can be avoided, whilst at the same time avoiding the negative dissolution properties of MgLAS₂, by producing a particle that contains both MgLAS₂ and NaLAS in a very specific ratio.

### SUMMARY OF THE INVENTION

The present invention provides a solid linear alkyl benzene sulphonate anionic detersive surfactant particle suitable for use in a laundry detergent composition, wherein the particle comprises from greater than 50wt% to 100wt% of a polycationic salt of linear alkyl benzene sulphonic acid comprising both magnesium and sodium cations, wherein the weight ratio of the magnesium salt of linear alkyl benzene sulphonic acid to the sodium salt of linear alkyl benzene sulphonic acid is in the range of from 0.6:1 to 9:1.

### DETAILED DESCRIPTION OF THE INVENTION

### Solid linear alkyl benzene sulphonate anionic detersive surfactant particle

The solid linear alkyl benzene sulphonate anionic detersive surfactant particle is suitable for use in a laundry detergent composition. The particle comprises from greater than 50wt% to 100wt% of a polycationic salt of linear alkyl benzene sulphonic acid comprising both magnesium and sodium cations. The weight ratio of the magnesium salt of linear alkyl benzene sulphonic acid to the sodium salt of linear alkyl benzene sulphonic acid is in the range of from 0.6:1 to 9:1.

Preferably, the particle comprises from 60wt% to 99wt%, or from 70wt% to 97wt%, or from 80wt% to 95wt% of the polycationic salt of linear alkyl benzene sulphonic acid.

The particle may comprise inorganic salt. The particle may comprise from above 0wt% to 40wt% inorganic salts. If present, the inorganic salt may be present at a level of from above 0wt% to 40wt%, or from 1wt% to 40wt%.

The particle may comprise from above 0wt% to 20wt% polymer. If present, the polymer may be present at a level of from above 0wt% to 20wt%, or from 1wt% to 20wt%.

The particle can be any suitable particulate form. Suitable forms include spray-dried particle, agglomerate, noodle, needle, ring, flake. A preferred form is a flake.

### Polycationic salt of linear alkyl benzene sulphonic acid

The polycationic salt of linear alkyl benzene sulphonic acid comprises both magnesium and sodium cations. The weight ratio of the magnesium salt of linear alkyl benzene sulphonic acid to the sodium salt of linear alkyl benzene sulphonic acid is in the range of from 0.6:1 to 9:1, preferably from 0.8:1 to 9:1, preferably from 0.9:1 to 7:1, preferably from 1:1 to 5:1.

Preferably, the linear alkyl benzene sulphonic acid has a 2-phenyl isomer content of from 15wt% to 20wt%.

### Inorganic Salt

Any suitable inorganic salt can be used.

Suitable inorganic salts are selected from: carbonate salts, chloride salts, magnesium salts, silicate salts, sulphate salts, zeolite salts, and any combination thereof.

Preferred inorganic salts are selected from: magnesium carbonate, magnesium sulphate, sodium carbonate, sodium sulphate, and any combination thereof.

### Polymer

Any suitable polymer can be used.

Suitable polymers are selected from: modified polysaccharide polymers, polycarboxylate polymers, polyethyleneglycol polymers, polyethylene imine polymers, silicone polymers, terephthalate polymers, other polyester polymers, and any combination thereof.

Preferred polymers are selected from: cellulosic polymer, polycarboxylate polymer, polyethyleneglycol polymer, silicone polymers, terephthalate polymer, and any combination thereof.

Suitable polymers are selected from modified polyamine polymers, modified polysaccharide polymers, polyalkylene oxide polymers, polycarboxylate polymers, silicone polymers, terephthalate polymers, other polyester polymers, and any combination thereof.

Preferably, the polymer is selected from polyamine polymers, modified polysaccharide polymers, polyalkylene oxide polymers, polycarboxylate polymers, and any combination thereof, most preferably, polycarboxylate polymers.

### Modified Polyamine Polymers

Suitable modified polyamine polymers comprise a polyamine core structure and a plurality of alkoxylate groups attached to the core structure. The polyamine core structure includes polyalkyleneimine, and linear or branched oligoamine.

The polyamine core structure and the alkoxylate groups attached to the core structure can be further derivatized. For example, the polyamine core structure can be further partly or completely quaternized with C₁-C₃₀ linear or branched alkyl, more preferably C₁-C₁₀ or even C₁-C₅ linear or branched alkyl, most preferably methyl. The alkoxylate group can be further sulphated, sulphonated and/or substituted with an amino functional group.

Suitable modified polyamine dispersing agent includes ethoxylated polyethyleneimine (EPEI). EPEI are effective dispersing agent for hydrophilic stains, especially hydrophilic particulate stain such as clay.

Preferably, the EPEI comprises a polyethyleneimine backbone having weight average molecular weight of between 100g/mol and 2000g/mol, preferably between 200g/mol and 1500g/mol, more preferably between 300g/mol and 1000g/mol, even more preferably between 400g/mol and 800g/mol, most preferably between 500g/mol and 700g/mol, preferably about 600. The ethoxylation chains within the EPEI may be from 200g/mol to 2000g/mol weight average molecular weight, preferably from 400g/mol to 1500g/mol weight average molecular weight, more preferably from 600g/mol to 1000g/mol weight average molecular weight, most preferably about 880g/mol weight average molecular weight per ethoxylated chain. The ethoxylation chains within the EPEI have on average 5 to 40, preferably 10 to 30, more preferably 15 to 25, even more preferably 18 to 22, most preferably about 20 ethoxy units per ethoxylation chain. The EPEI may have a total weight average molecular weight of from 5000g/mol to 20000g/mol, preferably from 7500g/mol to 17500g/mol, more preferably from 10000g/mol to 15000g/mol, even more preferably from 12000g/mol to 13000g/mol, most preferably about 12700g/mol. A preferred example is polyethyleneimine core (with average molecular weight about 600g/mol) ethoxylated to 20 EO groups per NH. Suitable EPEI this type includes Sokalan HP20 available from BASF, Lutensol FP620 from BASF. Examples of available polyethyleneimine ethoxylates also include those prepared by reacting ethylene oxide with Epomine SP-006 manufactured by Nippon Shokubai.

The EPEI may comprise polyethyleneimine having an average molecular weight (Mw) ranging from 1800 to 5000 g/mol (prior to ethoxylation), and the polyoxyethylene side chains may have an average of from 25 to 40 ethoxy units per side chain bonded to the polyethyleneimine backbone.

Suitable modified polyamine polymers include amphiphilic alkoxylated polyalkyleneimine polymer. These polymers have balanced hydrophilic and hydrophobic properties such that they remove grease and body soil particles from surfaces, and keep the particles suspended in washing liquor. Suitable amphiphilic water-soluble alkoxylated polyalkyleneimine polymers comprise polyalkyleneimine core, preferable polyethyleneimine core, and alkoxylate group connected to the core. Suitable alkoxylate groups have the structure:

^{∗}-[A²-O]ₘ₋[CH₂-CH₂-O]ₙ-[A³-O]ₚ-R (V)

wherein:
"*" in each case denotes one-half of bond to the nitrogen atom of the core.
A² is in each case independently selected from 1,2-propylene, 1,2-butylene, and 1,2-isobutylene.
A³ is 1,2-propylene.
R is in each case independently selected from hydrogen and C₁-C₄-alkyl, preferably hydrogen.
m has an average value in the range of from 0 to 2, preferably 0.
n has an average value in the range of 5 to 50.
p has an average value in the range of 3 to 50.

Suitable alkoxylated polyalkyleneimine polymers have a degree of quaterization ranging from 0 to 50, preferably from 0 to 20, and more preferably from 0 to 10.

A preferred alkoxylated polyalkyleneimine polymer is polyethyleneimine (MW = 600) modified with 24 ethoxylate groups per -NH and 16 propoxylate groups per -NH. Another preferred alkoxylated polyalkyleneimine polymer is polyethyleneimine (MW = 600) modified with 10 ethoxylate groups per -NH and 7 propoxylate groups per -NH.

Suitable alkoxylated polyalkyleneimine polymers include Sokalan HP30 Booster available from BASF.

Suitable modified polyamine polymers includes zwitterionic polyamines. Suitable zwitterionic polyamines have the structure: wherein:
R is each independently C₃-C₂₀ linear or branched alkylene.
R¹ is an anionic unit-capped polyalkyleneoxy unit having the formula: -(R²O)ₓR³.
R² is C₂-C₄ linear or branched alkylene, preferably C₂ (ethylene).
R³ is hydrogen, an anionic unit, and mixtures thereof, in which not all R³ groups are hydrogen, preferably wherein R³ anionic units are selected from -(CH₂)ₚCO₂M; -(CH₂)_{q}SO₃M; - (CH₂)_{q}OSO₃M; -(CH₂)_{q}CH(SO₃M)-CH₂SO₃M; -(CH₂)_{q}CH(OSO₃M)CH₂OSO3M; - (CH₂)_{q}CH(SO₃M)CH₂SO₃M; -(CH₂)ₚPO₃M; -PO₃M ;-SO₃M and mixtures thereof; wherein M is hydrogen or a water soluble cation, preferably selected from sodium, potassium, ammonium, and mixtures thereof and in sufficient amount to satisfy charge balance.
x is from 5 to 50, preferably from 10 to 40, even more preferably from 15 to 30, most preferably from 20 to 25.
Q is a quaternizing unit selected from the group consisting of C₁-C₃₀ linear or branched alkyl, C₆-C₃₀ cycloalkyl, C₇-C₃₀ substituted or unsubstituted alkylenearyl, and mixtures thereof, preferably C₁-C₃₀ linear or branched alkyl, even more preferably C₁-C₁₀ or even C₁-C₅ linear or branched alkyl, most preferably methyl; the degree of quaternization preferably is more than 50%, more preferably more than 70%, even more preferably more than 90%, most preferably about 100.
X⁻ is an anion present in sufficient amount to provide electronic neutrality, preferably a water-soluble anion selected from the group consisting of chlorine, bromine, iodine, methyl sulfate, and mixtures thereof, more preferably chloride.
n is from 0 to 8, preferably 0 to 4, preferably 0 to 2, most preferably 0.

A suitable zwitterionic polyamine having the following general structure: bis((C₂H₅O)(C₂H₄O)n)(CH₃)-N⁺-CₓH₂ₓ-N⁺-(CH₃)-bis((C₂H₅O)(C₂H₄O)n), wherein n = from 20 to 30, and x = from 3 to 8, or sulphated or sulphonated variants thereof.

A particular preferred zwitterionic polyamine is available from BASF as Lutensit Z96 polymer (zwitterionic hexamethylene diamine according to below formula: 100% quaternized and about 40% of the polyethoxy (EO₂₄) groups are sulfonated).

Another suitable zwitterionic polyamine is amphoterically-modified oligopropyleneimine ethoxylates.

### Modified Polysaccharide Polymers

Various polysaccharides can be useful as starting material for chemical modification to make modified polysaccharide polymers, including cellulose, starch, guar, dextran, polyglucan, chitin, curdlan, xylose, inulin, pullulan, locust bean gum, cassia gum, tamarind gum (xyloglucan), xanthan gum, amylose, amylopectin, scleroglucan and any combination thereof.

The most common type of modified polysaccharide is modified cellulose.

Modified cellulose polymers include anionic modified cellulose polymers which been modified with functional groups that contain negative charge. Suitable anionic modified cellulose polymers include carboxyalkyl cellulose, such as carboxymethyl cellulose. The carboxymethyl cellulose may have a degree of carboxymethyl substitution of from about 0.5 to about 0.9, and a molecular weight from about 80,000 Da to about 300,000 Da. Suitable carboxymethylcellulose include Finnfix^{®} series sold by CP Kelco or Nouryon, which include Finnfix^{®} GDA, a hydrophobically modified carboxymethylcellulose, e.g., the alkyl ketene dimer derivative of carboxymethylcellulose sold under the tradename Finnfix^{®} SH1, or the blocky carboxymethylcellulose sold under the tradename Finnfix^{®}V. Other suitable anionic modified cellulose polymers include sulphoalkyl cellulose and sulfoethyl cellulose.

Modified cellulose polymers also include nonionic modified cellulose polymers which have been modified by a functional group that does not contain any charge. Suitable nonionic modified cellulose polymers include alkyl cellulose, hydroxyalkyl cellulose, hydroxyalkyl alkylcellulose, alkylalkoxyalkyl cellulose. Suitable nonionic modified cellulose polymers also include nonionic cellulose carbamates, and nonionic 6-desoxy-6-amino-celluloses derivative. Examples of alkyl cellulose include methyl cellulose (MC), ethyl cellulose (EC), etc. Suitable ethyl celluloses are sold under tradename Ethocel^{™} by Dow Chemicals, DuPont, or IFF. Examples of hydroxyalkyl celluloses include hydroxyethyl cellulose (HEC) and hydroxypropyl cellulose (HPC). Suitable HECs are sold under tradename Natrosol^{™} hydroxyethylcellulose by Ashland, such as Natrosol^{™} 250 with different grades available which have a total molar substitution (MS) of 2.5. Suitable HECs are also sold under tradename CELLOSIZE^{™} Hydroxyethyl Cellulose by Dow Chemicals. Suitable HPCs are sold under tradename Klucel^{™} by Ashland. Example of hydroxyalkyl alkylcellulose include hydroxypropyl methylcellulose (HPMC), suitable HPMC are sold under tradename Methocel^{™} with different grades available by Dow Chemicals, DuPont or IFF, and under tradename Benecel^{™} by Ashland.

Modified cellulose polymers also include cationic modified cellulose polymers which been modified by functional group that contain cationic charge. Suitable cationic modified celluloses include quaternized hydroxyethyl cellulose (Polyquaternium-10), which is available under the tradename of Ucare by Dow Chemical, such as Ucare LR400, Ucare LR30M, Ucare JR125, Ucare JR400, etc. Suitable cationic modified cellulose polymers also include quaternized hydroxyethyl cellulose (HEC) polymers with cationic substitution of trimethyl ammonium and dimethyldodecyl ammonium (Polyquaternium-67), which are available under the tradename SoftCAT by Dow Chemical, such as SoftCAT SK, SoftCAT SK-MH, SoftCAT SX, SoftCAT SL. Other suitable cationic modified celluloses include those sold under tradename SupraCare^{™} by Dow Chemical, such as SupraCare^{™} 150, SupraCare^{™} 133, SupraCare^{™} 212. Suitable cationic modified cellulose polymers also include those modified with cationic group and a hydrophobic group.

Another suitable type of modified polysaccharide is modified guar. The modified guar can be nonionic modified, anionic modified, and/or cationic modified. Suitable nonionic modified guar includes hydroxypropyl guar, such as N-Hance^{™} HP40 and HP40S guar available from Ashland. Suitable example of modified guar also include carboxymethyl hydroxypropyl guar (CMHPG) which is anionic and nonionic modified, such as Galactasol^{™} available from Ashland. Suitable modified guar also includes cationic modified guar, such as guar hydroxypropyltrimonium chloride, which is available from by Ashland as AquaCat^{™} CG518 cationic solution, AquaCat^{™} PF618 cationic solution, N-Hance^{™} 3000, 3196, 3215, BF-13, BF-17, C261, C261N, CG13, CCG45. Other cationic modified guar polymers are available from Solvay as Jaguar^{®} C 162, Excel, Excel SGI, Optima, C 13 S, C 13 SH, C14 S, C-17, LS SGI, C-500 STD. Other nonionic and/or anionic modified guar include for example Jaguar^{®} HP 105 (Hydroxypropyl Guar gum), Jaguar^{®} SOFT and HP-120 COS (Carboxymethyl Hydroxypropyl Guar Gum).

Suitable modified polysaccharide polymers also include modified starch. Examples of modified starch include carboxylate ester of starch, esterification product of starch with e.g., C₆-C₂₄ alk(en)yl succinic anhydride;and starch maleates (starch react with maleic acid anhydride). Examples of modified starch also include, but not limit to, acetylated starch, acetylated distarch adipate, distarch phosphate, hydroxypropyl starch, hydroxy propyl distarch phosphate, phosphated distarch ohosphate, acetylated distarch phosphate, starch sodium octenyl succinate.

Suitable modified polysaccharide polymers also include polymers based on other polysaccharide, such as cationic dextran polymers, the cationic dextran polymers are commercially available under brand name CDC, CDC-L, CDC-H by Meito Sangyo.

Suitable modified polysaccharide polymers also include polymers based on polyglucans. Suitable modified polyglucans are based on alpha 1,3-polyglucans and/or 1,6-polyglucans. Preferably, the modified polyglucans can be cationic modified, such as cationic modified alpha 1,3-polyglucan, such as cationic modified alpha 1,6-polyglucans. Another class of preferred modified polyglucans can be hydrophobic and/or hydrophilic modified. Polyglucan esters are especially preferred due to their performance and biodegradability profiles.

Other suitable polysaccharide polymers include those based on inulin. Example of modified inulin include carboxymethyl group modified inulin (CMI), suitable CMI are Carboxyline series sold by Cosun Beet Company, including Carboxyline 25-40D, Carboxyline 25 D Powder, Carboxyline 20 LS D Powder, Carboxyline 25, Carboxyline 25-30 UP. Example of modified inulin also include cationic modified inulin, suitable cationic modified inulins include the Quatin series sold by Cosun Beet Company, including Quatin 350, Quatin 380 and Quatin 1280 which are characterized by different degree of substitution (DS), cationic density (meq/g) and molecular weight (g/mol).

Suitable modified polysaccharide polymers also include polymers based on other polysaccharide, such as xylose carbamates, carboxy or sulfo-alkylated pullulan, carboxy- or sulfo-alkylated chitosan, and any combination thereof.

### Polyalkylene Oxide Polymers

Suitable polyalkylene oxide polymers include poly (ethylene oxide). Preferably the poly (ethylene oxide) has a molecular weight from 1000 to 10000, more preferably from 2000 to 9000, more preferably from 3000 to 8500, most preferably from 4000 to 8000 such as 5000, 6000, 7000.

Suitable polyalkylene oxide polymers include graft polymers. Suitable graft polymers can be based on polyalkylene oxide Suitable polymers comprise polyalkylene oxide backbone (A) as a graft base and polymeric sidechains (B) grafted thereon. The polymeric sidechains (B) are obtainable by polymerization of at least one vinyl ester monomer. The polyalkylene oxide backbone (A) is obtainable by polymerization of at least one monomers selected from the group of ethylene oxide, 1 ,2-propylene oxide, 1 ,2-butylene oxide, 2,3-butylene oxide, 1 ,2-pentene oxide or 2,3-pentene oxide. Such graft polymers are known as effective soil suspension polymers for hydrophobic and hydrophilic stains, surfactant boosters, and sometimes as dye transfer inhibitors.

Suitable graft polymers include amphiphilic graft co-polymer comprising polyethylene glycol backbone (A) as a graft base, and at least one pendant sidechains (B) selected from polyvinyl acetate, polyvinyl alcohol and mixtures thereof. A preferred graft polymer of this type is Sokalan HP22 available from BASF.

Suitable graft polymers are amphiphilic graft polymers based on water-soluble polyalkylene oxides (A) as a graft base and side chains formed by polymerization of a vinyl ester component (B), said polymers typically having an average of < one graft site per 50 alkylene oxide units and mean molar masses M typically of from 3 000 to 100 000. One specific preferred graft polymer of this type is polyvinyl acetate grafted polyethylene oxide copolymer having a polyethylene oxide as graft base and multiple polyvinyl acetate side chains. The molecular weight of the polyethylene oxide backbone is typically about 6000 and the weight ratio of the polyethylene oxide to polyvinyl acetate is typically about 40 to 60 and typically no more than 1 grafting point per 50 ethylene oxide units. The most preferred polymer of this type is available from BASF as Sokalan PG101.

Suitable graft polymers include graft polymers comprising a block copolymer backbone (A) as a graft base, wherein said block copolymer backbone (A) is obtainable by polymerization of at least two monomers selected from the group of ethylene oxide, 1 ,2-propylene oxide, 1 ,2-butylene oxide, 2,3-butylene oxide, 1 ,2-pentene oxide or 2,3-pentene oxide, wherein the number (x) of individual blocks within the block copolymer backbone (A) is an integer, wherein x is typically from 2 to 10 and preferably 3 to 5, and (B) polymeric sidechains grafted onto the block copolymer backbone, wherein said polymeric sidechains (B) are obtainable by polymerization of at least one vinyl ester monomer. These polymers have improved biodegradation profiles.

Suitable graft polymers include graft polymers comprising a polyalkylene oxide backbone (A) which has a number average molecular weight of from about 1000 to about 20,000 Daltons and is based on ethylene oxide, propylene oxide, or butylene oxide; and side chains derived from N-vinylpyrrolidone (B), and side chains derived from vinyl ester (C) derived from a saturated monocarboxylic acid containing from 1 to 6 carbon atoms and/or a methyl or ethyl ester of acrylic or methacrylic acid.

### Polycarboxylate Polymers

Polycarboxylate polymers typically comprise at least one carboxy group-containing monomer. The carboxy group-containing monomers are typically selected from acrylic acid, methacrylic acid, fumaric acid, maleic acid, itaconic acid, aconitic acid, mesaconic acid, citraconic acid, methylenemalonic acid, salts thereof, anhydrides thereof, and any combination thereof.

Suitable polycarboxylate polymers include polyacrylate homopolymer having a molecular weight of from 4,000 Da to 9,000 Da, or from 6,000 Da to 9,000 Da. Other suitable carboxylate polymers include copolymers of acrylic acid (and/or methacrylic acid) and maleic acid having a molecular weight of from 50,000 Da to 120,000 Da, or from 60,000 Da to 80,000 Da. The polyacrylate homopolymer and copolymer of acrylic acid (and/or methacrylic acid) and maleic acid are commercially available as Acusol 445 and 445N, Acusol 531, Acusol 463, Acusol 448, Acusol 460, Acusol 465, Acusol 497, Acusol 490 from Dow Chemicals, and as Sokalan CP 5, Sokalan CP 7, Sokalan CP 45, and Sokalan CP 12S from BASF.

Suitable polycarboxylate polymers also include polyitaconate homopolymers, such as Itaconix^{®} DSP 2K^{™} sold by Itaconix, and Amaze SP available from Nouryon.

Suitable polycarboxylate polymers also include co-polymers comprising carboxy group-containing monomers and one or more sulfonate or sulfonic group-containing monomers. The sulfonate or sulfonic group containing monomers are typically selected from 2-acrylamido-2-methyl-1-propanesulfonic acid (AMPS), 2-methacrylamido-2-methyl-1-propanesulfonic acid, 3-methacrylamido-2-hydroxy-propanesulfonic acid, ally sulfonic acid, methallysulfonic acid, 3-allyloxy-2-hydroxy-1-propanesulfonic acid, 2-methyl-2-propenen-1-sulfonic acid, styrenesulfonic acid, vinylsulfonic acid, 3-sulfopropyl acrylate, 3-sulfopropylmethacrylate, sulfomethylacrylamide, sulfomethylmethacrylamide and water soluble salts thereof.

Suitable polymers may comprise maleic acid, acrylic acid, and 3-allyloxy-2-hydroxy-1-propanesulfonic acid. Suitable polymers may comprise acrylic acid and 2-acrylamido-2-methylpropane sulfonate, such as those sold under tradename Acusol 588 by Dow Chemicals, Sokalan CP50 by BASF, Aquatreat AR-545, Versaflex 310 and Versaflex 310-37 by Nouryon.

Suitable polymers include poly(itaconic acid-co-AMPS) sodium salt, such as Itaconix^{®} TSI^{™} 322 and Itaconix^{®} CHT^{™} 122 available from Itaconix.

Suitable polymers also includes those comprising other structure units in addition to the sulfonate or sulfonic group group-containing monomers and carboxy group-containing monomers. Suitable additional monomers are ether bond-containing monomers represented by formula (1) and (2) below: wherein in Formula (1):
R₀ represents a hydrogen atom or CH₃ group.
R represents a CH₂ group, CH₂CH₂ group or single bond.
x represents a number 0-50, preferably 0-20, more preferably 0-5 (provided x represents a number 1-5 when R is a single bond).
R₁ is a hydrogen atom or C₁ to C₂₀ organic group.
wherein in Formula (2):
   R₀ represents a hydrogen atom or CH₃ group.
   R represents a CH₂ group, CH₂CH₂ group or single bond.
   x represents a number 0-5.
   R₁ is a hydrogen atom or C₁ to C₂₀ organic group.

A specific preferred polymer comprises structure units derived from 1 to 49 wt% of 1-(allyloxy)-3-butoxypropan-2-ol, from 50 to 98 wt% acrylic acid or methacrylic acid, and from 1 to 49 wt% of 3-allyloxy-2-hydroxy-1-propanesulfonic acid, and the has a weight average molecular weight of from about 20,000 to about 60,000. a specific preferred polymer of this type comprises structure units derived from 1 to 10 wt% of 1-(allyloxy)-3-butoxypropan-2-ol, from 70 to 89 wt% acrylic acid or methacrylic acid, and from 10 to 20 wt% of 3-allyloxy-2-hydroxy-1-propanesulfonic acid, and the has a weight average molecular weight of from about 30,000 to about 60,000. Herein, 1-(allyloxy)-3-butoxypropan-2-ol is a preferred monomer as represented by formula (2) when R₀ is H, R is CH₂, x is 0, and R₁ is n-butyl (C₄-alkyl).

Suitable polycarboxylate polymers also include co-polymers comprising carboxy group-containing monomers and other suitable monomers. Other suitable monomers are selected from esters and/or amide of the carboxy group-containing monomers, such as C₁-C₂₀ alkyl ester of acrylic acid; alkylene; vinyl ethers, such as methyl vinyl ether, styrene and any mixtures thereof. One specific preferred polymer family of this type is sold under tradename Gantrez by Ashland, which includes Gantrez An (alternating co-polymer of methyl vinyl ether and maleic anhydride), Gantrez S (alternating co-polymer of methyl vinyl ether and maleic acid), Gantrez ES (alternating co-polymer of methyl vinyl ether and maleic acid ester), Gantrez MS (alternating co-polymer of methyl vinyl ether and maleic acid salt).

Suitable polycarboxylate polymers also include polyepoxy succinic acid polymers (PESA). A most preferred polyepoxy succinic acid polymer can be identified using CAS number: 51274-37-4, or 109578-44-1. Suitable polyepoxy succinic acid polymers are commercially available from various suppliers, such as Aquapharm Chemicals Pvt. Ltd (commercial name: Maxinol 600); Shandong Taihe Water Treatment Technologies Co., Ltd (commercial name: PESA), and Sirius International (commercial name: Briteframe PESA).

Suitable polycarboxylate polymers may comprise a monomer having at least one aspartic acid group or a salt thereof, this polymer comprises at least 25 mol%, 40 mol%, or 50 mol%, of said monomer. A preferabed example is sodium salt of poly(aspartic acid) having a molecular weight of from 2000 to 3000 g/mol which is avilable as Baypure^{®} DS 100 from Lanxess. Suitable polyaspartates can be further modified.

### Terephthalate Polymers

Suitable terephthalate polymers are terephthalate-derived polyester polymers, which comprise structure unit (I) and/or (II):

(I) -[(OCHR¹-CHR²)ₐ-O-OC-Ar-CO-]_{d}

(II) -[(OCHR³-CHR⁴)_{b}-O-OC-sAr-CO-]ₑ

wherein:
a, b are from 1 to 200.
d, e are from 1 to 50.
Ar is independently selected from 1,4-substituted phenylene, and 1,3-substituted phenylene.
sAr is 1,3-substituted phenylene substituted in position 5 with -SO₃M; wherein M is a counterion selected from Na, Li, K, Mg/2, Ca/2, Al/3, ammonium, mono-, di-, tri-, or tetraalkylammonium wherein the alkyl groups are C₁-C₁₈ alkyl or C₂-C₁₀ hydroxyalkyl, or mixtures thereof.
R¹, R², R³, R⁴ are independently selected from H or C₁-C₁₈ n-alkyl or iso-alkyl; preferably selected from H or C₁ alkyl.

Optionally, the polymer may further comprises one or more terminal group (III) derived from polyalkylene glycolmonoalkylethers, preferably selected from structure (IV-a)

-O-[C₂H₄-O]_{c}-[C₃H₆-O]_{d}-[C₄H₈-O]ₑ-R₇ (IV-a)

wherein:
R₇ is a linear or branched C₁₋₃₀ alkyl, C₂-C₃₀ alkenyl, or a cycloalkyl group with 5 to 9 carbon atoms, or a C₈-C₃₀ aryl group, or a C₆-C₃₀ arylalkyl group; preferably C₁₋₄ alkyl, more preferably methyl.
c, d and e are, based on molar average, a number independently selected from 0 to 200, where the sum of c+d+e is from 2 to 500.
wherein the [C₂H₄-O], [C₃H₆-O] and [C₄H₈-O] groups of the terminal group (IV-a) may be arranged blockwise, alternating, periodically and/or statistically, preferably blockwise and/or statistically, either of the [C₂H₄-O], [C₃H₆-O] and [C₄H₈-O] groups of the terminal group (IV-a) can be linked to -R₇ and/or -O. Preferably, [C₃H₆-O] group is linked to -O, and the -O is further connected to -OC-Ar-CO- or -OC-sAr-CO-.

Optionally, the polymer may further comprise one or more anionic terminal unit (IV) and/or (V) as described in EP3222647. Where M is a counterion selected from Na⁺, Li⁺, K⁺, ½ Mg²⁺, ½ Ca²⁺, 1/3 Al³⁺, ammonium, mono-, di-, tri-, or tetraalkylammonium wherein the alkyl groups are C₁-C₁₈ alkyl or C₂-C₁₀ hydroxyalkyl, or mixtures thereof.

-O-CH₂CH₂-SO₃M (IV)

Optionally, the polymer may comprise crosslinking multifunctional structural unit which having at least three functional groups capable of the esterification reaction. The functional which may be for example acid -, alcohol -, ester -, anhydride - or epoxy groups, etc.

Optionally, other di- or polycarboxylic acids or their salts or their (di)alkylesters can be used in the polyesters, such as, naphthalene-1,4-dicarboxylic acid, naphthalene-2,6,-dicarboxylic acid, tetrahydrophthalic acid, trimellitic acid, diphenoxyethane-4,4'-dicarboxylic acid, diphenyl-4,4'-dicarboxylic acid, 2,5-furandicarboxylic acid, adipic acid, sebacic acid, decan-1,10-dicarboxylic acid, fumaric acid, succinic acid, 1,4-cyclohexanedicarboxylic acid, cyclohexanediacetic acid, glutaric acid, azelaic acid, or their salts or their (di)alkyl esters, preferably their (C₁-C₄)-(di)alkyl esters and more preferably their (di)methyl esters, or mixtures thereof.

One type of preferred polyester polymers are nonionic polyester polymers which do not comprise the above structure unit (II). A particular preferred nonionic terephthalate-derived polymer has a structure according to formula below: wherein:
R₅ and R₆ are independently selected from H or CH₃. More preferably, one of the R₅ and R₆ is H, and another is CH₃.
c, d are, based on molar average, a number independently selected from 0 to 200, where the sum of c+d is from 2 to 400.

More preferably, d is from 0 to 50, c is from 1 to 200.

More preferably, d is 1 to 10, c is 5 to 150.
R₇ is C₁₋C₄ alkyl and more preferably methyl.
N is, based on molar average, from 1 to 50.

One example of most preferred above suitable terephthalate-derived nonionic polymers has one of the R₅ and R₆ is H, and another is CH₃; d is 0; c is from 5-100 and R₇ is methyl, and n is from 3-10.

Other suitable terephthalate-derived polyester polymers can be end capped. The end capping group of these SRPs are typically selected from:

X-(OC₂H₄)ₙ-(OC₃H₆)ₘ-

wherein, X is C₁-C₄ alkyl and preferably methyl, the -(OC₂H₄) groups and the -(OC₃H₆) groups are arranged blockwise and the block consisting of the -(OC₃H₆) groups is bound to a COO group, n is based on a molar average a number of from 40 to 50, m is based on a molar average a number of from 1 to 10 and preferably of from 1 to 7.

The polyester may or may not be biodegradable, preferred soil release polymers are readily biodegradable.

Example of suitable polyesters include TexCare^{®} series supplied by Clariant, including nonionic polymers Texcare^{®} SRN 100, SRN 170, SRN 170 C, SRN 170 Terra, SRN 172, SRN 240, SRN 260, SRN 260 life, SRN 260 SG Terra, SRN LTL50, SRN 300, SRN 325; and anionic polymers TexCare^{®} SRA 100, SRA 300, SRA300 F. Example of suitable polymers also include REPEL-O-TEX^{®} line of polymers supplied by Rhodia/Solvay, including the nonionic polymer REPEL-O-TEX^{®} Crystal, Crystal PLUS, Crystal NAT, SRP6; and the anionic polymer REPEL-O-TEX^{®} SF-2. Other examples of polymers includes the WeylClean^{®} series of polymers supplied by WeylChem, including nonionic polymers WeylClean^{®} PLN1, PLN2; and anionic polymers WeylClean^{®} PSA1. Other examples of polymers are Marloquest^{®} polymers, such as Marloquest^{®} SL, HSCB, L235M, U, B, and G82, supplied by Sasol. Suitable polymers include Sorez 100 (from ISP or Ashland).

### Other Polyester Polymers

Suitable other polyester polymers include polyester soil release polymers derived from bio-based 2,5-furandicarboxylic acid and derivatives thereof.

### Laundry Detergent Composition.

The laundry detergent composition comprises the solid linear alkyl benzene sulphonate anionic detersive surfactant particle.

Typically, the laundry detergent composition is a fully formulated laundry detergent composition, not a portion thereof such as a spray-dried, extruded or agglomerate particle that only forms part of the laundry detergent composition. Typically, the solid composition comprises a plurality of chemically different particles, such as spray-dried base detergent particles and/or agglomerated base detergent particles and/or extruded base detergent particles, in combination with one or more, typically two or more, or five or more, or even ten or more particles selected from: surfactant particles, including surfactant agglomerates, surfactant extrudates, surfactant needles, surfactant noodles, surfactant flakes; phosphate particles; zeolite particles; silicate salt particles, especially sodium silicate particles; carbonate salt particles, especially sodium carbonate particles; polymer particles such as carboxylate polymer particles, cellulosic polymer particles, starch particles, polyester particles, polyamine particles, terephthalate polymer particles, polyethylene glycol particles; aesthetic particles such as coloured noodles, needles, lamellae particles and ring particles; enzyme particles such as protease granulates, amylase granulates, lipase granulates, cellulase granulates, mannanase granulates, pectate lyase granulates, xyloglucanase granulates, bleaching enzyme granulates and co- granulates of any of these enzymes, preferably these enzyme granulates comprise sodium sulphate; bleach particles, such as percarbonate particles, especially coated percarbonate particles, such as percarbonate coated with carbonate salt, sulphate salt, silicate salt, borosilicate salt, or any combination thereof, perborate particles, bleach activator particles such as tetra acetyl ethylene diamine particles and/or alkyl oxybenzene sulphonate particles, bleach catalyst particles such as transition metal catalyst particles, and/or isoquinolinium bleach catalyst particles, pre-formed peracid particles, especially coated pre-formed peracid particles; filler particles such as sulphate salt particles and chloride particles; clay particles such as montmorillonite particles and particles of clay and silicone; flocculant particles such as polyethylene oxide particles; wax particles such as wax agglomerates; silicone particles, brightener particles; dye transfer inhibition particles; dye fixative particles; perfume particles such as perfume microcapsules and starch encapsulated perfume accord particles, or pro-perfume particles such as Schiff base reaction product particles; hueing dye particles; chelant particles such as chelant agglomerates; and any combination thereof.

Suitable laundry detergent compositions comprise a detergent ingredient selected from: detersive surfactant, such as anionic detersive surfactants, non-ionic detersive surfactants, cationic detersive surfactants, zwitterionic detersive surfactants and amphoteric detersive surfactants; polymers, such as carboxylate polymers, soil release polymer, anti-redeposition polymers, cellulosic polymers and care polymers; bleach, such as sources of hydrogen peroxide, bleach activators, bleach catalysts and pre-formed peracids; photobleach, such as such as zinc and/or aluminium sulphonated phthalocyanine; enzymes, such as proteases, amylases, cellulases, lipases; zeolite builder; phosphate builder; co-builders, such as citric acid and citrate; carbonate, such as sodium carbonate and sodium bicarbonate; sulphate salt, such as sodium sulphate; silicate salt such as sodium silicate; chloride salt, such as sodium chloride; brighteners; chelants; hueing agents; dye transfer inhibitors; dye fixative agents; perfume; silicone; fabric softening agents, such as clay; flocculants, such as polyethyleneoxide; suds supressors; and any combination thereof.

Suitable laundry detergent compositions may have a low buffering capacity. Such laundry detergent compositions typically have a reserve alkalinity to pH 9.5 of less than 5.0gNaOH/100g. These low buffered laundry detergent compositions typically comprise low levels of carbonate salt.

Detersive Surfactant: Suitable detersive surfactants include anionic detersive surfactants, non-ionic detersive surfactant, cationic detersive surfactants, zwitterionic detersive surfactants and amphoteric detersive surfactants. Suitable detersive surfactants may be linear or branched, substituted or un-substituted, and may be derived from petrochemical material or biomaterial.

Anionic detersive surfactant: Suitable anionic detersive surfactants include sulphonate and sulphate detersive surfactants.

Suitable sulphonate detersive surfactants include methyl ester sulphonates, alpha olefin sulphonates, alkyl benzene sulphonates, especially alkyl benzene sulphonates, preferably C₁₀₋₁₃ alkyl benzene sulphonate. Suitable alkyl benzene sulphonate (LAS) is obtainable, preferably obtained, by sulphonating commercially available linear alkyl benzene (LAB); suitable LAB includes low 2-phenyl LAB, other suitable LAB include high 2-phenyl LAB, such as those supplied by Sasol under the tradename Hyblene^{®}.

Suitable sulphate detersive surfactants include alkyl sulphate, preferably C₈₋₁₈ alkyl sulphate, or predominantly C₁₂ alkyl sulphate.

A preferred sulphate detersive surfactant is alkyl alkoxylated sulphate, preferably alkyl ethoxylated sulphate, preferably a C₈₋₁₈ alkyl alkoxylated sulphate, preferably a C₈₋₁₈ alkyl ethoxylated sulphate, preferably the alkyl alkoxylated sulphate has an average degree of alkoxylation of from 0.5 to 20, preferably from 0.5 to 10, preferably the alkyl alkoxylated sulphate is a C₈₋₁₈ alkyl ethoxylated sulphate having an average degree of ethoxylation of from 0.5 to 10, preferably from 0.5 to 5, more preferably from 0.5 to 3 and most preferably from 0.5 to 1.5.

The alkyl sulphate, alkyl alkoxylated sulphate and alkyl benzene sulphonates may be linear or branched, substituted or un-substituted, and may be derived from petrochemical material or biomaterial.

Other suitable anionic detersive surfactants include alkyl ether carboxylates.

Suitable anionic detersive surfactants may be in salt form, suitable counter-ions include sodium, calcium, magnesium, amino alcohols, and any combination thereof. A preferred counter-ion is sodium.

Non-ionic detersive surfactant: Suitable non-ionic detersive surfactants are selected from the group consisting of: C₈-C₁₈ alkyl ethoxylates, such as, NEODOL^{®} non-ionic surfactants from Shell; C₆-C₁₂ alkyl phenol alkoxylates wherein preferably the alkoxylate units are ethyleneoxy units, propyleneoxy units or a mixture thereof; C₁₂-C₁₈ alcohol and C₆-C₁₂ alkyl phenol condensates with ethylene oxide/propylene oxide block polymers such as Pluronic^{®} from BASF; alkylpolysaccharides, preferably alkylpolyglycosides; methyl ester ethoxylates; polyhydroxy fatty acid amides; ether capped poly(oxyalkylated) alcohol surfactants; and mixtures thereof.

Suitable non-ionic detersive surfactants are alkylpolyglucoside and/or an alkyl alkoxylated alcohol.

Suitable non-ionic detersive surfactants include alkyl alkoxylated alcohols, preferably C₈₋₁₈ alkyl alkoxylated alcohol, preferably a C₈₋₁₈ alkyl ethoxylated alcohol, preferably the alkyl alkoxylated alcohol has an average degree of alkoxylation of from 1 to 50, preferably from 1 to 30, or from 1 to 20, or from 1 to 10, preferably the alkyl alkoxylated alcohol is a C₈₋₁₈ alkyl ethoxylated alcohol having an average degree of ethoxylation of from 1 to 10, preferably from 1 to 7, more preferably from 1 to 5 and most preferably from 3 to 7. The alkyl alkoxylated alcohol can be linear or branched, and substituted or un-substituted.

Suitable nonionic detersive surfactants include secondary alcohol-based detersive surfactants.

Cationic detersive surfactant: Suitable cationic detersive surfactants include alkyl pyridinium compounds, alkyl quaternary ammonium compounds, alkyl quaternary phosphonium compounds, alkyl ternary sulphonium compounds, and mixtures thereof.

Preferred cationic detersive surfactants are quaternary ammonium compounds having the general formula:

(R)(R₁)(R₂)(R₃)N⁺ X⁻

wherein, R is a linear or branched, substituted or unsubstituted C₆₋₁₈ alkyl or alkenyl moiety, R₁ and R₂ are independently selected from methyl or ethyl moieties, R₃ is a hydroxyl, hydroxymethyl or a hydroxyethyl moiety, X is an anion which provides charge neutrality, preferred anions include: halides, preferably chloride; sulphate; and sulphonate.

Zwitterionic detersive surfactant: Suitable zwitterionic detersive surfactants include amine oxides and/or betaines.

Polymer: Suitable polymers include carboxylate polymers, soil release polymers, anti-redeposition polymers, cellulosic polymers, care polymers and any combination thereof.

Carboxylate polymer: The composition may comprise a carboxylate polymer, such as a maleate/acrylate random copolymer or polyacrylate homopolymer. Suitable carboxylate polymers include: polyacrylate homopolymers having a molecular weight of from 4,000 Da to 9,000 Da; maleate/acrylate random copolymers having a molecular weight of from 50,000 Da to 100,000 Da, or from 60,000 Da to 80,000 Da.

Another suitable carboxylate polymer is a co-polymer that comprises: (i) from 50 to less than 98 wt% structural units derived from one or more monomers comprising carboxyl groups; (ii) from 1 to less than 49 wt% structural units derived from one or more monomers comprising sulfonate moieties; and (iii) from 1 to 49 wt% structural units derived from one or more types of monomers selected from ether bond-containing monomers represented by formulas (I) and (II): formula (I):
wherein in formula (I), R₀ represents a hydrogen atom or CH₃ group, R represents a CH₂ group, CH₂CH₂ group or single bond, X represents a number 0-5 provided X represents a number 1-5 when R is a single bond, and R₁ is a hydrogen atom or C₁ to C₂₀ organic group;
wherein in formula (II), R₀ represents a hydrogen atom or CH₃ group, R represents a CH₂ group, CH₂CH₂ group or single bond, X represents a number 0-5, and R₁ is a hydrogen atom or C₁ to C₂₀ organic group.

It may be preferred that the polymer has a weight average molecular weight of at least 50kDa, or even at least 70kDa.

Soil release polymer: The composition may comprise a soil release polymer. A suitable soil release polymer has a structure as defined by one of the following structures (I), (II) or (III):

(I) -[(OCHR¹-CHR²)ₐ-O-OC-Ar-CO-]_{d}

(II) -[(OCHR³-CHR⁴)_{b}-O-OC-sAr-CO-]ₑ

(III) -[(OCHR⁵-CHR⁶)_{c}-OR⁷]_{f}

wherein:
a, b and c are from 1 to 200;
d, e and f are from 1 to 50;
Ar is a 1,4-substituted phenylene;
sAr is 1,3-substituted phenylene substituted in position 5 with SO₃Me;
Me is Li, K, Mg/2, Ca/2, Al/3, ammonium, mono-, di-, tri-, or tetraalkylammonium wherein the alkyl groups are C₁-C₁₈ alkyl or C₂-C₁₀ hydroxyalkyl, or mixtures thereof;
R¹, R², R³, R⁴, R⁵ and R₆ are independently selected from H or C₁-C₁₈ n- or iso-alkyl; and
R₇ is a linear or branched C₁-C₁₈ alkyl, or a linear or branched C₂-C₃₀ alkenyl, or a cycloalkyl group with 5 to 9 carbon atoms, or a C₈-C₃₀ aryl group, or a C₆-C₃₀ arylalkyl group.

Suitable soil release polymers are sold by Clariant under the TexCare^{®} series of polymers, e.g. TexCare^{®} SRN240 and TexCare^{®} SRA300. Other suitable soil release polymers are sold by Solvay under the Repel-o-Tex^{®} series of polymers, e.g. Repel-o-Tex^{®} SF2 and Repel-o-Tex^{®} Crystal.

Anti-redeposition polymer: Suitable anti-redeposition polymers include polyethylene glycol polymers and/or polyethyleneimine polymers.

Suitable polyethylene glycol polymers include random graft co-polymers comprising: (i) hydrophilic backbone comprising polyethylene glycol; and (ii) hydrophobic side chain(s) selected from the group consisting of: C₄-C₂₅ alkyl group, polypropylene, polybutylene, vinyl ester of a saturated C₁-C₆ mono-carboxylic acid, C₁-C₆ alkyl ester of acrylic or methacrylic acid, and mixtures thereof. Suitable polyethylene glycol polymers have a polyethylene glycol backbone with random grafted polyvinyl acetate side chains. The average molecular weight of the polyethylene glycol backbone can be in the range of from 2,000 Da to 20,000 Da, or from 4,000 Da to 8,000 Da. The molecular weight ratio of the polyethylene glycol backbone to the polyvinyl acetate side chains can be in the range of from 1: 1 to 1:5, or from 1: 1.2 to 1:2. The average number of graft sites per ethylene oxide unit can be less than 0.02, or less than 0.016, the average number of graft sites per ethylene oxide unit can be in the range of from 0.010 to 0.018, or the average number of graft sites per ethylene oxide unit can be less than 0.010, or in the range of from 0.004 to 0.008.

Suitable polyethylene glycol polymers are described in WO08/007320.

A suitable polyethylene glycol polymer is Sokalan HP22.

Cellulosic polymer: Suitable cellulosic polymers are selected from alkyl cellulose, alkyl alkoxyalkyl cellulose, carboxyalkyl cellulose, alkyl carboxyalkyl cellulose, sulphoalkyl cellulose, more preferably selected from carboxymethyl cellulose, methyl cellulose, methyl hydroxyethyl cellulose, methyl carboxymethyl cellulose, and mixures thereof.

Suitable carboxymethyl celluloses have a degree of carboxymethyl substitution from 0.5 to 0.9 and a molecular weight from 100,000 Da to 300,000 Da.
Suitable carboxymethyl celluloses have a degree of substitution greater than 0.65 and a degree of blockiness greater than 0.45, e.g. as described in WO09/154933.

Care polymers: Suitable care polymers include cellulosic polymers that are cationically modified or hydrophobically modified. Such modified cellulosic polymers can provide anti-abrasion benefits and dye lock benefits to fabric during the laundering cycle. Suitable cellulosic polymers include cationically modified hydroxyethyl cellulose.

Other suitable care polymers include dye lock polymers, for example the condensation oligomer produced by the condensation of imidazole and epichlorhydrin, preferably in ratio of 1:4:1. A suitable commercially available dye lock polymer is Polyquart^{®} FDI (Cognis).

Other suitable care polymers include amino-silicone, which can provide fabric feel benefits and fabric shape retention benefits.

Bleach: Suitable bleach includes sources of hydrogen peroxide, bleach activators, bleach catalysts, pre-formed peracids and any combination thereof. A particularly suitable bleach includes a combination of a source of hydrogen peroxide with a bleach activator and/or a bleach catalyst.

Source of hydrogen peroxide: Suitable sources of hydrogen peroxide include sodium perborate and/or sodium percarbonate.

Bleach activator: Suitable bleach activators include tetra acetyl ethylene diamine and/or alkyl oxybenzene sulphonate.

Bleach catalyst: The composition may comprise a bleach catalyst. Suitable bleach catalysts include oxaziridinium bleach catalysts, transistion metal bleach catalysts, especially manganese and iron bleach catalysts. A suitable bleach catalyst has a structure corresponding to general formula below: wherein R¹³ is selected from the group consisting of 2-ethylhexyl, 2-propylheptyl, 2-butyloctyl, 2-pentylnonyl, 2-hexyldecyl, n-dodecyl, n-tetradecyl, n-hexadecyl, n-octadecyl, isononyl, iso-decyl, iso-tridecyl and iso-pentadecyl.

Pre-formed peracid: Suitable pre-form peracids include phthalimido-peroxycaproic acid.

Enzymes: Suitable enzymes include lipases, proteases, cellulases, amylases and any combination thereof.

Protease: Suitable proteases include metalloproteases and/or serine proteases. Examples of suitable neutral or alkaline proteases include: subtilisins (EC 3.4.21.62); trypsin-type or chymotrypsin-type proteases; and metalloproteases. The suitable proteases include chemically or genetically modified mutants of the aforementioned suitable proteases.

Suitable commercially available protease enzymes include those sold under the trade names Alcalase^{®}, Savinase^{®}, Primase^{®}, Durazym^{®}, Polarzyme^{®}, Kannase^{®}, Liquanase^{®}, Liquanase Ultra^{®}, Savinase Ultra^{®}, Ovozyme^{®}, Neutrase^{®}, Everlase^{®} and Esperase^{®} by Novozymes A/S (Denmark), those sold under the tradename Maxatase^{®}, Maxacal^{®}, Maxapem^{®}, Preferenz P^{®} series of proteases including Preferenz^{®} P280, Preferenz^{®} P281, Preferenz^{®} P2018-C, Preferenz^{®} P2081-WE, Preferenz^{®} P2082-EE and Preferenz^{®} P2083-A/J, Properase^{®}, Purafect^{®}, Purafect Primer Purafect Ox^{®}, FN3^{®} , FN4^{®}, Excellase^{®} and Purafect OXP^{®} by DuPont, those sold under the tradename Opticlean^{®} and Optimase^{®} by Solvay Enzymes, those available from Henkel/ Kemira, namely BLAP (sequence shown in Figure 29 of US 5,352,604 with the folowing mutations S99D + S101 R + S103A + V104I + G159S, hereinafter referred to as BLAP), BLAP R (BLAP with S3T + V4I + V199M + V205I + L217D), BLAP X (BLAP with S3T + V4I + V205I) and BLAP F49 (BLAP with S3T + V4I + A194P + V199M + V205I + L217D) - all from Henkel/Kemira; and KAP (Bacillus alkalophilus subtilisin with mutations A230V + S256G + S259N) from Kao.

A suitable protease is described in WO11/140316 and WO11/072117.

Amylase: Suitable amylases are derived from AA560 alpha amylase endogenous to Bacillus sp. DSM 12649, preferably having the following mutations: R118K, D183*, G184*, N195F, R320K, and/or R458K. Suitable commercially available amylases include Stainzyme^{®}, Stainzyme^{®} Plus, Natalase, Termamyl^{®}, Termamyl^{®} Ultra, Liquezyme^{®} SZ, Duramyl^{®}, Everest^{®} (all Novozymes) and Spezyme^{®} AA, Preferenz S^{®} series of amylases, Purastar^{®} and Purastar^{®} Ox Am, Optisize^{®} HT Plus (all Du Pont).
A suitable amylase is described in WO06/002643.

Cellulase: Suitable cellulases include those of bacterial or fungal origin. Chemically modified or protein engineered mutants are also suitable. Suitable cellulases include cellulases from the genera *Bacillus, Pseudomonas, Humicola, Fusarium, Thielavia, Acremonium,* e.g., the fungal cellulases produced from *Humicola insolens, Myceliophthora thermophila* and *Fusarium oxysporum.*

Commercially available cellulases include Celluzyme^{®}, Carezyme^{®}, and Carezyme^{®} Premium, Celluclean^{®} and Whitezyme^{®} (Novozymes A/S), Revitalenz^{®} series of enzymes (Du Pont), and Biotouch^{®} series of enzymes (AB Enzymes). Suitable commercially available cellulases include Carezyme^{®} Premium, Celluclean^{®} Classic. Suitable cellulases are described in WO07/144857 and WO10/056652.

Lipase: Suitable lipases include those of bacterial, fungal or synthetic origin, and variants thereof. Chemically modified or protein engineered mutants are also suitable. Examples of suitable lipases include lipases from *Humicola* (synonym *Thermomyces*), e.g., from *H. lanuginosa* (*T. lanuginosus*)*.*

The lipase may be a "first cycle lipase", e.g. such as those described in WO06/090335 and WO13/116261. In one aspect, the lipase is a first-wash lipase, preferably a variant of the wild-type lipase from Thermomyces lanuginosus comprising T231R and/or N233R mutations. Preferred lipases include those sold under the tradenames Lipex^{®}, Lipolex^{®} and Lipoclean^{®} by Novozymes, Bagsvaerd, Denmark.

Other suitable lipases include: Liprl 139, e.g. as described in WO2013/171241; and TfuLip2, e.g. as described in WO2011/084412 and WO2013/033318.

Other enzymes: Other suitable enzymes are bleaching enzymes, such as peroxidases/oxidases, which include those of plant, bacterial or fungal origin and variants thereof. Commercially available peroxidases include Guardzyme^{®} (Novozymes A/S). Other suitable enzymes include choline oxidases and perhydrolases such as those used in Gentle Power Bleach^{™}.

Other suitable enzymes include pectate lyases sold under the tradenames X-Pect^{®}, Pectaway^{®} (from Novozymes A/S, Bagsvaerd, Denmark) and PrimaGreen^{®} (DuPont) and mannanases sold under the tradenames Mannaway^{®} (Novozymes A/S, Bagsvaerd, Denmark), and Mannastar^{®} (Du Pont).

Zeolite builder: The composition may comprise zeolite builder. The composition may comprise from 0wt% to 5wt% zeolite builder, or 3wt% zeolite builder. The composition may even be substantially free of zeolite builder; substantially free means "no deliberately added". Typical zeolite builders include zeolite A, zeolite P and zeolite MAP.

Phosphate builder: The composition may comprise phosphate builder. The composition may comprise from 0wt% to 5wt% phosphate builder, or to 3wt%, phosphate builder. The composition may even be substantially free of phosphate builder; substantially free means "no deliberately added". A typical phosphate builder is sodium tri-polyphosphate.

Carbonate salt: The composition may comprise carbonate salt. The composition may comprise from 0wt% to 10wt% carbonate salt, or to 5wt% carbonate salt. The composition may even be substantially free of carbonate salt; substantially free means "no deliberately added". Suitable carbonate salts include sodium carbonate and sodium bicarbonate.

Silicate salt: The composition may comprise silicate salt. The composition may comprise from 0wt% to 10wt% silicate salt, or to 5wt% silicate salt. A preferred silicate salt is sodium silicate, especially preferred are sodium silicates having a Na₂O:SiO₂ ratio of from 1.0 to 2.8, preferably from 1.6 to 2.0.

Sulphate salt: A suitable sulphate salt is sodium sulphate.

Brightener: Suitable fluorescent brighteners include: di-styryl biphenyl compounds, e.g. Tinopal^{®} CBS-X, di-amino stilbene di-sulfonic acid compounds, e.g. Tinopal^{®} DMS pure Xtra and Blankophor^{®} HRH, and Pyrazoline compounds, e.g. Blankophor^{®} SN, and coumarin compounds, e.g. Tinopal^{®} SWN.
Preferred brighteners are: sodium 2 (4-styryl-3-sulfophenyl)-2H-napthol[1,2-d]triazole, disodium 4,4'-bis{[(4-anilino-6-(N methyl-N-2 hydroxyethyl)amino 1 ,3,5- triazin-2-yl)];amino}stilbene-2-2' disulfonate, disodium 4,4'-bis{[(4-anilino-6-morpholino-1,3,5-triazin-2-yl)]amino} stilbene-2-2' disulfonate, and disodium 4,4'- bis(2-sulfostyryl)biphenyl. A suitable fluorescent brightener is C.I. Fluorescent Brightener 260, which may be used in its beta or alpha crystalline forms, or a mixture of these forms.

Chelant: The composition may also comprise a chelant selected from: diethylene triamine pentaacetate, diethylene triamine penta(methyl phosphonic acid), ethylene diamine-N'N'-disuccinic acid, ethylene diamine tetraacetate, ethylene diamine tetra(methylene phosphonic acid) and hydroxyethane di(methylene phosphonic acid). A preferred chelant is ethylene diamine-N'N'-disuccinic acid (EDDS) and/or hydroxyethane diphosphonic acid (HEDP). The composition preferably comprises ethylene diamine-N'N'- disuccinic acid or salt thereof. Preferably the ethylene diamine-N'N'-disuccinic acid is in S,S enantiomeric form. Preferably the composition comprises 4,5-dihydroxy-m-benzenedisulfonic acid disodium salt. Preferred chelants may also function as calcium carbonate crystal growth inhibitors such as: 1-hydroxyethanediphosphonic acid (HEDP) and salt thereof; N,N-dicarboxymethyl-2-aminopentane-1,5-dioic acid and salt thereof; 2-phosphonobutane-1,2,4-tricarboxylic acid and salt thereof; and combination thereof.

Hueing agent: Suitable hueing agents include small molecule dyes, typically falling into the Colour Index (C.I.) classifications of Acid, Direct, Basic, Reactive (including hydrolysed forms thereof) or Solvent or Disperse dyes, for example classified as Blue, Violet, Red, Green or Black, and provide the desired shade either alone or in combination. Preferred such hueing agents include Acid Violet 50, Direct Violet 9, 66 and 99, Solvent Violet 13 and any combination thereof.

Many hueing agents are known and described in the art which may be suitable for the present invention, such as hueing agents described in WO2014/089386.

Suitable hueing agents include phthalocyanine and azo dye conjugates, such as described in WO2009/069077.

Suitable hueing agents may be alkoxylated. Such alkoxylated compounds may be produced by organic synthesis that may produce a mixture of molecules having different degrees of alkoxylation. Such mixtures may be used directly to provide the hueing agent, or may undergo a purification step to increase the proportion of the target molecule. Suitable hueing agents include alkoxylated bis-azo dyes, such as described in WO2012/054835, and/or alkoxylated thiophene azo dyes, such as described in WO2008/087497 and WO2012/166768.

The hueing agent may be incorporated into the detergent composition as part of a reaction mixture which is the result of the organic synthesis for a dye molecule, with optional purification step(s). Such reaction mixtures generally comprise the dye molecule itself and in addition may comprise un-reacted starting materials and/or by-products of the organic synthesis route. Suitable hueing agents can be incorporated into hueing dye particles, such as described in WO 2009/069077.

Dye transfer inhibitors: Suitable dye transfer inhibitors include polyamine N-oxide polymers, copolymers of N-vinylpyrrolidone and N-vinylimidazole, polyvinylpyrrolidone, polyvinyloxazolidone, polyvinylimidazole and mixtures thereof. Preferred are poly(vinyl pyrrolidone), poly(vinylpyridine betaine), poly(vinylpyridine N-oxide), poly(vinyl pyrrolidone-vinyl imidazole) and mixtures thereof. Suitable commercially available dye transfer inhibitors include PVP-K15 and K30 (Ashland), Sokalan^{®} HP165, HP50, HP53, HP59, HP56K, HP56, HP66 (BASF), Chromabond^{®} S-400, S403E and S-100 (Ashland).

Perfume: Suitable perfumes comprise perfume materials selected from the group: (a) perfume materials having a ClogP of less than 3.0 and a boiling point of less than 250°C (quadrant 1 perfume materials); (b) perfume materials having a ClogP of less than 3.0 and a boiling point of 250°C or greater (quadrant 2 perfume materials); (c) perfume materials having a ClogP of 3.0 or greater and a boiling point of less than 250°C (quadrant 3 perfume materials); (d) perfume materials having a ClogP of 3.0 or greater and a boiling point of 250°C or greater (quadrant 4 perfume materials); and (e) mixtures thereof.

It may be preferred for the perfume to be in the form of a perfume delivery technology. Such delivery technologies further stabilize and enhance the deposition and release of perfume materials from the laundered fabric. Such perfume delivery technologies can also be used to further increase the longevity of perfume release from the laundered fabric. Suitable perfume delivery technologies include: perfume microcapsules, pro-perfumes, polymer assisted deliveries, molecule assisted deliveries, fiber assisted deliveries, amine assisted deliveries, cyclodextrin, starch encapsulated accord, zeolite and other inorganic carriers, and any mixture thereof. A suitable perfume microcapsule is described in WO2009/101593.

Silicone: Suitable silicones include polydimethylsiloxane and amino-silicones. Suitable silicones are described in WO05075616.

Process for making the solid composition: Typically, the particles of the composition can be prepared by any suitable method. For example: spray-drying, agglomeration, extrusion and any combination thereof.

Typically, a suitable spray-drying process comprises the step of forming an aqueous slurry mixture, transferring it through at least one pump, preferably two pumps, to a pressure nozzle. Atomizing the aqueous slurry mixture into a spray-drying tower and drying the aqueous slurry mixture to form spray-dried particles. Preferably, the spray-drying tower is a counter-current spray-drying tower, although a co-current spray-drying tower may also be suitable.

Typically, the spray-dried powder is subjected to cooling, for example an air lift. Typically, the spray-drying powder is subjected to particle size classification, for example a sieve, to obtain the desired particle size distribution. Preferably, the spray-dried powder has a particle size distribution such that weight average particle size is in the range of from 300 micrometers to 500 micrometers, and less than 10wt% of the spray-dried particles have a particle size greater than 2360 micrometers.

It may be preferred to heat the aqueous slurry mixture to elevated temperatures prior to atomization into the spray-drying tower, such as described in WO2009/158162.

It may be preferred for anionic surfactant, such as linear alkyl benzene sulphonate, to be introduced into the spray-drying process after the step of forming the aqueous slurry mixture: for example, introducing an acid precursor to the aqueous slurry mixture after the pump, such as described in WO 09/158449.

It may be preferred for a gas, such as air, to be introduced into the spray-drying process after the step of forming the aqueous slurry, such as described in WO2013/181205.

It may be preferred for any inorganic ingredients, such as sodium sulphate and sodium carbonate, if present in the aqueous slurry mixture, to be micronized to a small particle size such as described in WO2012/134969.

Typically, a suitable agglomeration process comprises the step of contacting a detersive ingredient, such as a detersive surfactant, e.g. linear alkyl benzene sulphonate (LAS) and/or alkyl alkoxylated sulphate, with an inorganic material, such as sodium carbonate and/or silica, in a mixer. The agglomeration process may also be an in-situ neutralization agglomeration process wherein an acid precursor of a detersive surfactant, such as LAS, is contacted with an alkaline material, such as carbonate and/or sodium hydroxide, in a mixer, and wherein the acid precursor of a detersive surfactant is neutralized by the alkaline material to form a detersive surfactant during the agglomeration process.

Other suitable detergent ingredients that may be agglomerated include polymers, chelants, bleach activators, silicones and any combination thereof.

The agglomeration process may be a high, medium or low shear agglomeration process, wherein a high shear, medium shear or low shear mixer is used accordingly. The agglomeration process may be a multi-step agglomeration process wherein two or more mixers are used, such as a high shear mixer in combination with a medium or low shear mixer. The agglomeration process can be a continuous process or a batch process.

It may be preferred for the agglomerates to be subjected to a drying step, for example to a fluid bed drying step. It may also be preferred for the agglomerates to be subjected to a cooling step, for example a fluid bed cooling step.

Typically, the agglomerates are subjected to particle size classification, for example a fluid bed elutriation and/or a sieve, to obtain the desired particle size distribution. Preferably, the agglomerates have a particle size distribution such that weight average particle size is in the range of from 300 micrometers to 800 micrometers, and less than 10wt% of the agglomerates have a particle size less than 150 micrometers and less than 10wt% of the agglomerates have a particle size greater than 1200 micrometers.

It may be preferred for fines and over-sized agglomerates to be recycled back into the agglomeration process. Typically, over-sized particles are subjected to a size reduction step, such as grinding, and recycled back into an appropriate place in the agglomeration process, such as the mixer. Typically, fines are recycled back into an appropriate place in the agglomeration process, such as the mixer.

It may be preferred for ingredients such as polymer and/or non-ionic detersive surfactant and/or perfume to be sprayed onto base detergent particles, such as spray-dried base detergent particles and/or agglomerated base detergent particles. Typically, this spray-on step is carried out in a tumbling drum mixer.

Method of laundering fabric: The method of laundering fabric comprises the step of contacting the solid composition to water to form a wash liquor, and laundering fabric in said wash liquor. Typically, the wash liquor has a temperature of above 0°C to 90°C, or to 60°C, or to 40°C, or to 30°C, or to 20°C. The fabric may be contacted to the water prior to, or after, or simultaneous with, contacting the solid composition with water. Typically, the wash liquor is formed by contacting the laundry detergent to water in such an amount so that the concentration of laundry detergent composition in the wash liquor is from 0.2g/l to 20g/l, or from 0.5g/l to 10g/l, or to 5.0g/l. The method of laundering fabric can be carried out in a front-loading automatic washing machine, top loading automatic washing machines, including high efficiency automatic washing machines, or suitable hand-wash vessels._Typically, the wash liquor comprises 90 litres or less, or 60 litres or less, or 15 litres or less, or 10 litres or less of water. Typically, 200g or less, or 150g or less, or 100g or less, or 50g or less of laundry detergent composition is contacted to water to form the wash liquor.
Method of making the solid linear alkyl benzene sulphonate anionic detersive surfactant particle

The method obtains the polycationic salt of linear alkyl benzene sulphonic acid. The polycationic salt of linear alkyl benzene sulphonic acid is obtained by the process steps
(a) partially neutralizing a linear alkyl benzene sulphonic acid with a magnesium neutralizing agent to form a partially magnesium neutralized linear alkyl benzene sulphonic acid; and
(b) fully neutralizing the partially magnesium neutralized linear alkyl benzene sulphonic acid from step (a) with a sodium neutralizing agent to form the polycationic salt of linear alkyl benzene sulphonic acid comprising both magnesium and sodium cations.

Preferably, the magnesium neutralizing agent is selected from magnesium bicarbonate, magnesium carbonate, magnesium carbonate hydroxide magnesium hydroxide, and any combination thereof.

Preferably, the sodium neutralizing agent is selected from sodium bicarbonate, sodium carbonate, sodium hydroxide, and any combination thereof.

This process is a particularly effective way of making a particle of the present invention.

### EXAMPLES

### EXAMPLE 1

Eleven linear alkyl benzene sulphonate (LAS) anionic detersive surfactant flakes were made, each with a different ratio of magnesium linear alkyl benzene sulphonate (MgLAS₂) anionic detersive surfactant to sodium linear alkyl benzene sulphonate (NaLAS) anionic detersive surfactant.

All LAS flakes were made by drying pre-made LAS pastes. The LAS pastes were made by neutralization of linear alkyl benzene sulphonic acid (HLAS) with magnesium hydroxide (Mg(OH)₂) and/or sodium hydroxide (NaOH). For pastes and flakes that contain both MgLAS₂ and NaLAS, the order of addition of the hydroxide salts was MgOH₂ followed by NaOH to avoid MgOH₂ precipitation prior to full neutralization of the HLAS. The grade of HLAS used contained traces of sulphuric acid (H₂SO₄), which undergoes neutralization prior to HLAS due to its lower pKa value. The reactions that take place are thus:
Neutralization with Mg(OH)₂ only (Paste / Flake A below)
   1.

      H₂SO₄ + Mg(OH)₂ → MgSO₄ + 2 H₂O
   2.

      2 HLAS + Mg(OH)₂ → Mg(LAS)₂ + 2 H₂O
Neutralization with both Mg(OH)₂ and NaOH (Pastes / Flakes B-J below)
   1.

      H₂SO₄ + Mg(OH)₂ → MgSO₄ + 2 H₂O
   2.

      2 HLAS + Mg(OH)₂ → Mg(LAS)₂ + 2 H₂O
   3.

      HLAS + NaOH → NaLAS + H₂O
Neutralization with NaOH only (Paste / Flake K below)
   1.

      H₂SO₄ + 2 NaOH → Na₂SO₄ + 2 H₂O
   2.

      HLAS + NaOH → NaLAS + H₂O

All eleven pastes were made in beakers with overhead stirrers to accelerate and complete the neutralization reactions and paste homogenization. Impeller rotational velocities varied from 300 RPM to 1000 RPM depending on the observed evolving thickness of the paste as the HLAS was neutralized to LAS. For all pastes tabulated below, the order of addition is as follows:
For pastes that contain Mg(LAS)₂ (A-J):
   1. Water (liquid)
   2. Mg(OH)₂ (solid)
   3. HLAS (liquid)
   4. NaOH (aq.) (if present)
   5. Polycarboxylate polymer (liquid)
   6. Sodium sulphate (solid)
For the paste that does not contain Mg(LAS)₂ (K):
   1. Water (liquid)
   2. NaOH (aq.)
   3. HLAS (liquid)
   4. Polycarboxylate polymer (liquid)
   5. Sodium sulphate (solid)

**Table 1-A**

| Paste | A | B | C | D | E | F | G | H | I | J | K |
|---|---|---|---|---|---|---|---|---|---|---|---|
| MgLAS [%w] | 61.5 | 55.4 | 49.2 | 43.0 | 36.8 | 30.8 | 24.6 | 18.5 | 12.3 | 6.2 | 0.0 |
| NaLAS [%w] | 0.0 | 6.2 | 12.3 | 18.5 | 24.7 | 30.8 | 36.9 | 43.1 | 49.2 | 55.4 | 61.5 |
| Polycarboxylate [%w] | 1.0 | 1.0 | 1.0 | 1.0 | 1.0 | 1.0 | 1.0 | 1.0 | 1.0 | 1.0 | 1.0 |
| Sodium sulphate [%w] | 2.8 | 2.8 | 2.8 | 2.8 | 2.8 | 2.8 | 2.8 | 2.8 | 2.8 | 2.8 | 3.6 |
| Magnesium sulphate [%w] | 0.8 | 0.7 | 0.7 | 0.7 | 0.7 | 0.7 | 0.7 | 0.7 | 0.7 | 0.7 | 0.0 |
| Water [%w] | 33.0 | 33.0 | 33.0 | 33.0 | 33.0 | 33.0 | 33.0 | 33.0 | 33.0 | 33.0 | 33.0 |
| Unsulphonated alkylbenzene [%w] | 0.9 | 0.9 | 0.9 | 0.9 | 0.9 | 0.9 | 0.9 | 0.9 | 0.9 | 0.9 | 0.9 |
| Mass ratio (MgLAS₂/ NaLAS) [-] | - | 9.00 | 4.00 | 2.33 | 1.49 | 1.00 | 0.67 | 0.43 | 0.25 | 0.11 | 0.00 |

When made, the LAS pastes were applied and spread onto a silicone baking mat in layers with a thickness of up to 5 mm. The silicone baking mats with applied LAS pastes were then placed in an oven set to 110 °C and left to dry for 16 hours. After 16 hours, the LAS pastes were extracted from the silicone baking mats as large flakes. These large flakes were subsequently grated on a sieve with an aperture size of 1180 µm, optionally below which sieves with aperture sizes of 600 µm and 425 µm were present, with a pan at the bottom. As such, dried flakes with particle sizes of 0-425 µm, 425-600 µm, 600-1180 µm, and 0-1180 µm were obtained.

**Table 1-B**

| Flake | A | B | C | D | E | F | G | H | I | J | K |
|---|---|---|---|---|---|---|---|---|---|---|---|
| MgLAS [%w] | 90.0 | 81.0 | 72.0 | 62.9 | 53.9 | 45.0 | 36.1 | 27.1 | 18.0 | 9.0 | 0.0 |
| NaLAS [%w] | 0.0 | 9.0 | 18.0 | 27.1 | 36.1 | 45.0 | 53.9 | 62.9 | 72.0 | 81.0 | 90.0 |
| Polycarboxylate [%w] | 1.5 | 1.5 | 1.5 | 1.5 | 1.5 | 1.5 | 1.5 | 1.5 | 1.5 | 1.5 | 1.5 |
| Sodium sulphate [%w] | 4.1 | 4.1 | 4.1 | 4.1 | 4.1 | 4.1 | 4.1 | 4.2 | 4.2 | 4.2 | 5.2 |
| Magnesium sulphate [%w] | 1.1 | 1.1 | 1.1 | 1.1 | 1.1 | 1.1 | 1.1 | 1.1 | 1.1 | 1.1 | 0.0 |
| Water [%w] | < 2.0 | < 2.0 | < 2.0 | < 2.0 | < 2.0 | < 2.0 | < 2.0 | < 2.0 | < 2.0 | < 2.0 | < 2.0 |
| Unsulphonated alkylbenzene [%w] | 1.4 | 1.3 | 1.3 | 1.3 | 1.3 | 1.3 | 1.3 | 1.3 | 1.3 | 1.3 | 1.3 |
| Mass ratio (MgLAS₂/ NaLAS) [-] | - | 9.00 | 4.00 | 2.33 | 1.49 | 1.00 | 0.67 | 0.43 | 0.25 | 0.11 | 0.00 |

All eleven flakes were placed in unique unitized solid laundry detergent composition matrices, the composition of which is tabulated in Table 1-C. Each composition matrix was unitized via surrounding the composition matrix in non-woven polyvinyl alcohol. All eleven unitized solid laundry detergent composition matrices were placed in a climate chamber with conditions of 25 °C and 60% relative humidity for 12 weeks. After 12 weeks, each unitized matrix was assessed for the free-flowing nature of the solid laundry detergent composition inside of it. After the assessment, the relative humidity of the solid laundry detergent composition was measured to be (60 ± 2)% RH, thus indicating that equilibrium conditions were achieved.

**Table 1-C**

| Raw material | Raw material activity [%w] | Raw material fraction in composition [%w] |
|---|---|---|
| LAS flake | 90.0 | 45.4 |
| Sodium percarbonate | 87.6 | 30.2 |
| TAED | 92.0 | 9.00 |
| Zeolite | 80.0 | 3.45 |
| Polycarboxylate | 92.0 | 2.10 |
| Carboxymethyl cellulose | 65.0 | 1.80 |
| Sodium sulphate | 100.0 | 8.05 |

To assess the physical flow properties of the powder composition matrix after storage at 60% relative humidity, the non-woven polyvinyl alcohol was removed, and the powder was poured onto a sieve with an aperture size of 2 mm. After shaking the sieve for 30 seconds, the mass on the sieve was measured, and the mass passing through the sieve was measured. The results are tabulated in table 1-D.

As the powder in each unitized matrix contained 45.4%w LAS flake, any amount of powder on the 2 mm sieve less than 45.4%w implies that not all the LAS flake contributes to consolidated particles exceeding 2 mm in size. Therefore, the invention considers a flake which is present in any powder of which less than 45.4%w remains on the 2 mm sieve.

**Table 1-D**

| Flake | A | B | C | D | E | F | G | H | I | J | K |
|---|---|---|---|---|---|---|---|---|---|---|---|
| Mass ratio (MgLAS₂/ NaLAS) [-] | - | 9.00 | 4.00 | 2.33 | 1.49 | 1.00 | 0.67 | 0.43 | 0.25 | 0.11 | 0.00 |
| Mass on 2 mm sieve [g] | 2.1 | 3.9 | 7.0 | 5.8 | 8.2 | 16.5 | 19.1 | 29.8 | 30.9 | 33.9 | 43.7 |
| Mass through 2 mm sieve [g] | 44.0 | 42.1 | 38.4 | 41.0 | 37.3 | 29.1 | 25.1 | 17.9 | 17.2 | 13.6 | 3.1 |
| Fraction of powder on 2 mm sieve [%w] | 4.6 | 8.5 | 15.4 | 12.4 | 18.0 | 36.2 | 43.2 | 62.5 | 64.2 | 71.4 | 93.4 |

It was observed that flakes A, B, C, D, E, F, and G all resulted in the powder matrix they were a part of having less than 45.4% of their total mass left on the 2 mm sieve. Flakes H, I, J, and K all resulted in the powder matrix they were a part of having more than 45.4% of their total mass left on the 2 mm sieve.

### EXAMPLE 2

Two linear alkyl benzene sulphonate (LAS) anionic detersive surfactant flakes were made, following the process as described in EXAMPLE 1. For these flakes and their paste precursors, the polycarboxylate polymer was omitted. One of the flakes and its paste precursor used a HLAS source for which the unsulphonated linear alkylbenzene (LAB) precursor was classed as having a high level of 2-phenyl isomers, and the other flake used a HLAS source for which the LAB precursor was classed as having a low level of 2-phenyl isomers.

**Table 2-A**

| Paste | E-L2Ph | E-H2Ph |
|---|---|---|
| 2-phenyl isomer content [%w of total isomer mass] | 15-20 | 25-30 |
| MgLAS [%w] | 36.9 | 36.9 |
| NaLAS [%w] | 24.6 | 24.6 |
| Sodium sulphate [%w] | 3.8 | 3.8 |
| Magnesium sulphate [%w] | 0.7 | 0.7 |
| Water [%w] | 33.0 | 33.0 |
| Unsulphonated alkylbenzene [%w] | 0.9 | 0.9 |
| Mass ratio (MgLAS₂ / NaLAS) [-] | 1.49 | 1.49 |

**Table 2-B**

| Flake | E-L2Ph | E-H2Ph |
|---|---|---|
| 2-phenyl isomer content [%w of total isomer mass] | 15-20 | 25-30 |
| MgLAS [%w] | 54.0 | 54.0 |
| NaLAS [%w] | 36.0 | 36.0 |
| Sodium sulphate [%w] | 5.6 | 5.6 |
| Magnesium sulphate [%w] | 1.1 | 1.1 |
| Water [%w] | < 2.0 | < 2.0 |
| Unsulphonated alkylbenzene [%w] | 1.3 | 1.3 |
| Mass ratio (MgLAS₂ / NaLAS) [-] | 1.49 | 1.49 |

Two flakes were placed in unique unitized solid laundry detergent composition matrices, the composition of which is tabulated in Table 2-C. Each composition matrix was unitized via surrounding the composition matrix in non-woven polyvinyl alcohol. Both unitized solid laundry detergent composition matrices were placed in a climate chamber with conditions of 25 °C and 60% relative humidity for 14 weeks. After 14 weeks, each unitized matrix was assessed for the free-flowing nature of the solid laundry detergent composition inside of it. After the assessment, the relative humidity of the solid laundry detergent composition was measured to be (60 ± 2)% RH, thus indicating that equilibrium conditions were achieved.

**Table 2-C**

| Raw material | Raw material activity [%w] | Raw material fraction in composition [%w] |
|---|---|---|
| LAS flake | 90.0 | 45.4 |
| Sodium percarbonate | 87.6 | 30.2 |
| TAED | 92.0 | 9.00 |
| Zeolite | 80.0 | 3.45 |
| Polycarboxylate | 92.0 | 2.10 |
| Carboxymethyl cellulose | 65.0 | 1.80 |
| Sodium sulphate | 100.0 | 8.05 |

To assess the physical flow properties of the powder composition matrix after storage at 60% relative humidity, the non-woven polyvinyl alcohol was removed, and the powder was poured onto a sieve with an aperture size of 2 mm. After shaking the sieve for 30 seconds, the mass on the sieve was measured, and the mass passing through the sieve was measured. The results are tabulated in table 2-D.

**Table 2-D**

| Flake | E-L2Ph | E-H2Ph |
|---|---|---|
| 2-phenyl isomer content [%w of total isomer mass] | 15-20 | 25-30 |
| Mass ratio (MgLAS₂ / NaLAS) [-] | 1.49 | 1.49 |
| Mass on 2 mm sieve [g] | 10.7 | 21.7 |
| Mass through 2 mm sieve [g] | 38.0 | 28.3 |
| Fraction of powder on 2 mm sieve [%w] | 22.0 | 43.4 |

It was observed that the flake comprising the low-2-phenyl isomer perform particularly well.

### EXAMPLE 3

For flakes A, B, C, D, E, F, and K as prepared in EXAMPLE 1, dissolution kinetics were analyzed via UV-Visible spectrophotometry. For each measurement, 0.44 grams of "fresh" flake were dissolved into 800 mL of de-ionized water under mechanical stirring. A sample of each flake was left to stir for 24 hours, after which a wavelength-scan experiment was run, resulting in values for absorbance for each flake across a wavelength range of 190-400 nm. Table 3-A shows the absorbance (in Absorbance Units, A. U.) at a wavelength of 250 nm for each of the flakes.

**Table 3-A**

| Flake | UV-Visible absorbance at 250 nm [A. U.] |
|---|---|
| A | 0.46 |
| B | 0.51 |
| C | 0.53 |
| D | 0.54 |
| E | 0.55 |
| F | 0.54 |
| K | 0.54 |

A different sample of each flake was then measured for absorbance at a wavelength of 250 nm over a period of 10 minutes, at intervals 1, 2, 5 and 10 minutes. The measured absorbance values were then calculated as a percentage of the dissolution measured after 24 hours as tabulated in Table 3-A. The results are shown in Table 3-B.

**Table 3-B**

| | After stirring for 1 minutes | | After stirring for 2 minutes | | After stirring for 5 minutes | | After stirring for 10 minutes | |
|---|---|---|---|---|---|---|---|---|
| Flake | A* | D** | A* | D** | A* | D** | A* | D** |
| A | 0.13 | 29 | 0.28 | 61 | 0.20 | 43 | 0.23 | 50 |
| B | 0.17 | 34 | 0.23 | 45 | 0.28 | 54 | 0.32 | 61 |
| C | 0.19 | 37 | 0.27 | 50 | 0.34 | 64 | 0.38 | 71 |
| D | 0.21 | 38 | 0.32 | 60 | 0.40 | 74 | 0.41 | 76 |
| E | 0.23 | 42 | 0.34 | 62 | 0.41 | 75 | 0.42 | 77 |
| F | 0.20 | 36 | 0.29 | 54 | 0.38 | 69 | 0.41 | 76 |
| K | 0.39 | 73 | 0.43 | 80 | 0.47 | 86 | 0.50 | 93 |

| | | | | | | | | |
|---|---|---|---|---|---|---|---|---|
| * A = "UV-Visible spectrophotometry absorbance at 250 nm [A. U.]" ** D = "Percentage dissolution compared to dissolution at 24 hours per Table 3-A [%]" | | | | | | | | |

It was observed that after 10 minutes, flake B, C, D, E, F, and K have a dissolution percentage of at least 60% of their respective 24-hour dissolution values.

The dimensions and values disclosed herein are not to be understood as being strictly limited to the exact numerical values recited. Instead, unless otherwise specified, each such dimension is intended to mean both the recited value and a functionally equivalent range surrounding that value. For example, a dimension disclosed as "40 mm" is intended to mean "about 40 mm".

## Claims

1. A solid linear alkyl benzene sulphonate anionic detersive surfactant particle suitable for use in a laundry detergent composition, wherein the particle comprises from greater than 50wt% to 100wt% of a polycationic salt of linear alkyl benzene sulphonic acid comprising both magnesium and sodium cations, wherein the weight ratio of the magnesium salt of linear alkyl benzene sulphonic acid to the sodium salt of linear alkyl benzene sulphonic acid is in the range of from 0.6: 1 to 9:1.

2. A particle according to claim 1, wherein the weight ratio of the magnesium salt of linear alkyl benzene sulphonic acid to the sodium salt of linear alkyl benzene sulphonic acid is in the range of from 0.9: 1 to 7:1.

3. A particle according to any preceding claim, wherein the weight ratio of the magnesium salt of linear alkyl benzene sulphonic acid to the sodium salt of linear alkyl benzene sulphonic acid is in the range of from 1: 1 to 5: 1.

4. A particle according to any preceding claim, wherein the particle comprises from 80wt% to 95wt% of the polycationic salt of linear alkyl benzene sulphonic acid.

5. A particle according to any preceding claim, wherein the particle comprises from above 0wt% to 40wt% inorganic salts.

6. A particle according to claim 5, wherein the inorganic salt is selected from: carbonate salts, chloride salts, magnesium salts, silicate salts, sulphate salts, zeolite salts, and any combination thereof.

7. A particle according to any of claims 5-6, wherein the inorganic salt is selected from: magnesium carbonate, magnesium sulphate, sodium carbonate, sodium sulphate, and any combination thereof.

8. A particle according to any preceding claim, wherein the particle comprises from above 0wt% to 20wt% polymer.

9. A particle according to claim 8, wherein the polymer is selected from: modified polysaccharide polymers, polycarboxylate polymers, polyethyleneglycol polymers, polyethylene imine polymers, silicone polymers, terephthalate polymers, other polyester polymers, and any combination thereof.

10. A particle according to any preceding claim, wherein the linear alkyl benzene sulphonic acid has a 2-phenyl isomer content of from 15wt% to 20wt%.

11. A particle according to any preceding claim, wherein the particle is in the form of a flake.

12. A laundry detergent composition comprising a particle according to any preceding claim.

13. A method of making a particle according to any of claims 1-11, wherein the polycationic salt of linear alkyl benzene sulphonic acid is obtained by the process steps
(a) partially neutralizing a linear alkyl benzene sulphonic acid with a magnesium neutralizing agent to form a partially magnesium neutralized linear alkyl benzene sulphonic acid; and
(b) fully neutralizing the partially magnesium neutralized linear alkyl benzene sulphonic acid from step (a) with a sodium neutralizing agent to form the polycationic salt of linear alkyl benzene sulphonic acid comprising both magnesium and sodium cations.

14. A method according to claim 13, wherein the magnesium neutralizing agent is selected from magnesium bicarbonate, magnesium carbonate, magnesium carbonate hydroxide magnesium hydroxide, and any combination thereof.

15. A method according to any of claims 13-14, wherein the sodium neutralizing agent is selected from sodium bicarbonate, sodium carbonate, sodium hydroxide, and any combination thereof.
